

Patented July 23, 1929.

1,722,146

## UNITED STATES PATENT OFFICE.

WILLIAM IRBY, OF LYNN, MASSACHUSETTS, ASSIGNOR TO GENERAL ELECTRIC COMPANY, A CORPORATION OF NEW YORK.

### ELECTRODE.

No Drawing.

Application filed January 7, 1927. Serial No. 159,741.

My invention relates to electrodes for arc lamps, and more particularly to electrodes especially adapted for use in connection with the so-called luminous arc.

5 One of the objects of my invention is to provide an electrode of the ilmenite magnetite class, the operation of which is materially improved.

Flaming arc electrodes are commonly 10 made of a mixture of ilmenite, magnetite and chromite, together with a flux of sodium fluoride. I have found that the operation of such electrodes can be very materially improved by substituting the following mixture:

Per cent.

|                   |       |
|-------------------|-------|
| Ilmenite          | 69.0  |
| Magnetite         | 14.92 |
| Chromite          | 3.0   |
| 20 Ferro-titanium | 12.8  |
| Sodium fluoride   | 0.28  |

It will be understood, however, that I do not wish to be strictly limited to the exact proportions given, inasmuch as, in view of the disclosure, variations may be made in 25 the proportions without departing from the spirit of the invention or the scope of the claim contained herein.

What I claim as new, and desire to secure by Letters Patent of the United States, 30 is:

An electrode for an electric arc consisting of the following ingredients, in substantially the following proportions: ilmenite 69.0%, chromite 3.0%, magnetite 14.92%, 25 sodium fluoride 0.28% and ferro-titanium 12.8%.

In witness whereof, I have hereunto set my hand this 5th day of January, 1927.

WILLIAM IRBY.